

Patented Dec. 15, 1936

2,063,907

# UNITED STATES PATENT OFFICE

2,063,907

## METHOD OF DELUSTERING FABRIC

Camille Dreyfus, New York, N. Y., and Herbert Platt, Cumberland, Md., assignors to Celanese Corporation of America, a corporation of Delaware

No Drawing. Application September 1, 1928,  
Serial No. 303,602

4 Claims. (Cl. 28—1)

This invention relates to the treatment of textile materials containing organic derivatives of cellulose so as to subdue the luster of the same.

5 An object of our invention is to reduce the luster of textile materials containing organic derivatives of cellulose in such a manner that the deluster effect is comparatively permanent.

10 Another object of our invention is to deluster textile materials containing organic derivatives of cellulose by precipitating an opaque and insoluble salt in the textile material. Other objects of our invention will appear from the following detailed description.

15 Heretofore textile materials containing organic derivatives of cellulose, such as cellulose acetate, have been delustered by boiling water, wet steam or aqueous solutions of various reagents. However, the delustering effect produced by such processes is not permanent and such delustered fabrics regain all or part of their luster when they are ironed while damp or subjected to dry steam or other agencies. Obviously this tendency to reluster is a serious drawback.

20 25 We have found that a practically permanent subdued luster may be imparted to an organic derivative of cellulose material by precipitating an opaque insoluble salt throughout and within the fibres of the yarn of the organic ester of cellulose.

30 In accordance with our invention, we treat a textile material containing organic derivatives of cellulose with a solution of a salt of a metal that produces a white and opaque salt, which is itself a swelling agent for the organic derivatives of cellulose, or in the presence of a foreign swelling agent, and then treat the same with a solution that is adapted to precipitate the metal in the form of an opaque and white salt.

35 40 45 The textile material to be treated in accordance with our invention may be in the form of yarns in a suitable package such as in hanks, on bobbins, etc. However, we prefer to treat a fabric containing yarns of such organic derivatives of cellulose. The fabric may contain any organic derivatives of cellulose such as cellulose esters and cellulose ethers. Examples of cellulose esters are cellulose acetate, cellulose formate, cellulose propionate and cellulose butyrate, while examples of cellulose ethers are ethyl cellulose, methyl cellulose and benzyl cellulose. The fabric need not consist wholly of yarns of such organic derivatives but may also contain yarns of other material such as cotton, silk, wool, etc.

We have found that solutions of salts of the alkaline earth metals such as barium, calcium or strontium produce satisfactory results. The solutions of such salts may be of themselves swelling agents. Examples of such salts are 5 the sulfocyanides of barium or other alkaline earth metal. On the other hand, salts of such metals such as the chloride or chlorate of barium may be employed, which of themselves are not swelling agents. In this case the treating bath may also contain a swelling agent such as formic acid, acetic acid, acetone, etc. If desired, the textile material may be first treated with a bath containing these swelling agents and then with a bath containing the salts of the 10 alkaline earth metals.

15 After treatment with the solutions of the alkaline earth metals, the textile material is then treated with a solution that is adapted to precipitate the metal in the form of an 20 opaque and white salt. Suitable reagents for this purpose are aqueous solutions of sulphuric acid, phosphoric acid or the soluble salts of these acids such as the sulphates or phosphates of sodium, potassium, or ammonium. By treating 25 of the material in such baths, the sulphates or phosphates of barium, strontium or calcium are formed.

30 Because of the action of the swelling agent, the salts permeate throughout the fibres and 35 are generally retained therein so that when they are precipitated as insoluble salts they will not wash out. The textile materials produced by our invention have a subdued luster varying 40 depending on the concentration and time of treatment, and this deluster effect is permanent. Fabrics when treated by our invention may be ironed while damp or subjected to dry steam or other relustering agent without becoming relustered.

45 To obtain further desirable effects, the textile material to be treated by our invention may be partially saponified and particularly "intensely surface saponified." By this is meant treatment with alkaline solutions in such concentrations and in such manner that only the outer 50 layers of the fibres of cellulose ester material is saponified, while the inner core is preferably unaffected so that the safe ironing point is materially increased. This partial saponification step may be carried out on the textile material either prior to the delustering treatment or subsequent thereto.

The fabrics when treated in accordance with our invention have an affinity for organic derivatives of cellulose dyestuffs and basic dyestuffs, and also have an increased affinity for direct cotton colors and for acid colors.

In order further to illustrate our invention, the following specific examples are given.

*Example I*

10 A fabric consisting solely of yarns of cellulose acetate is treated for one hour at 70° C. in a 25° Tw. solution of barium thiocyanate. It is then treated for 20 minutes in the cold in a 1% solution of sulphuric acid, after which it is rinsed and dried. The fabric so treated is quite well delustered, which luster is not appreciably affected by ironing or washing.

*Example II*

20 A fabric consisting wholly of cellulose acetate is first treated for one hour at 50° C. in an aqueous solution containing 20% of formic acid, which acts as a swelling agent. It is then treated for one hour at 70° C. in a solution of barium chloride and is then treated for 20 minutes in the cold in a 1% aqueous solution of phosphoric acid and is then rinsed and dried. The fabric is satisfactory delustered and is not appreciably relustered by ironing, either wet or dry or by washing.

30 The fabric resulting from the treatments of the foregoing examples contains filaments wherein the barium compound, which is a pigment-like inorganic material, occurs as small particles submerged in and widely distributed throughout the mass of the filaments and the quantity and distribution of the particles is such as not to materially impair the continuity of the mass of the filaments. Moreover the amount of barium compound that becomes incorporated in the filaments is a small percentage of the mass of the filaments. Such barium compounds are inert to the action of chemicals used in the manufacture, dyeing and bleaching of the filaments or fabrics.

40 We are well aware of the fact that textile materials containing organic derivatives of cellulose, such as cellulose acetate, have been previously treated with salts of tin and the like for the purpose of weighting the same. Our invention is quite different from this weighting process, since

the materials used for weighting are employed for a different purpose and therefore the weighted material has substantially the same luster as the original material, while the weight of the same is materially increased, whereas in our process the luster of the textile material is substantially subdued and the weight thereof is but slightly increased.

5 It is to be understood that the foregoing detailed description is given merely by way of illustration and that many variations may be made therein without departing from the spirit of this invention.

Having described our invention what we claim and desire to secure by Letters Patent is:

15 1. Method of treating fabric containing yarns of organic derivatives of cellulose comprising treating such fabric with a solution of barium sulphocyanide and then treating the fabric with a solution containing sulphate ions, whereby 20 barium sulphate is precipitated within the fibres of such yarn.

2. Method of treating fabric containing yarns of cellulose acetate comprising treating such fabric with a solution of barium sulphocyanide and 25 then treating the fabric with a solution containing sulphate ions, whereby barium sulphate is precipitated within the fibres of such yarn.

3. Method of treating fabric containing yarns of organic derivatives of cellulose comprising 30 treating such fabric with a solution of an alkaline earth metal sulphocyanide which is a swelling agent for the derivative of cellulose and then treating the fabric with a solution containing ions selected from the group consisting of sulphate and phosphate ions, whereby 35 an insoluble alkaline earth metal compound is precipitated within the fibres of such yarn.

4. Method of treating fabric containing yarns of cellulose acetate comprising treating such fabric with a solution of an alkaline earth metal sulphocyanide which is a swelling agent for the cellulose acetate and then treating the fabric with a solution containing ions selected from the group 40 consisting of sulphate and phosphate ions, where- 45 by an insoluble alkaline earth metal compound is precipitated within the fibres of such yarn.

CAMILLE DREYFUS.  
HERBERT PLATT.